

March 7, 1961

P. E. McGARRY

2,973,864

PROCESS FOR BENEFICIATION OF ASPHALTITE MATERIAL

Filed Jan. 6, 1955



Inventor:  
Philip E. McGarry  
By: Everett F. Smith  
Attorney

## PROCESS FOR BENEFICIATION OF ASPHALTITE MATERIAL

Phillip E. McGarry, Lakeland, Fla., assignor to International Minerals & Chemical Corporation, a corporation of New York

Filed Jan. 6, 1955, Ser. No. 480,289

9 Claims. (Cl. 209—166)

This invention relates to the beneficiation of uranium-bearing asphaltite ore. More particularly, it relates to the beneficiation of rock impregnated with bituminous material bearing uranium components. Still more particularly, it relates to a flotation process for dolomitic formations impregnated with uranium-bearing bitumens.

Asphaltite or bituminous rocks such as gilsonite, grahamite, wurtzite, etc., are mined in various sections of the United States. In the western states there are numerous occurrences of dolomite formations containing uranium-bearing asphaltite material. The percentage of asphaltite material present in these ores is relatively small, generally less than about 10% and usually being of the order of about 1% to about 5%. The uranium analyzed as  $U_3O_8$  is present in quantities generally of the order of about 0.01% to about 0.06% by weight of the ore. Chemical recovery methods are not economically feasible for use on such low grade uranium ore materials.

It is an object of this invention to provide a relatively inexpensive method of recovering the bituminous material and the uranium compounds associated therewith in a concentrated form.

It is still another object of this invention to provide an economical feasible method for preparation of an asphaltite concentrate useful as a feed material for chemical extraction processes for the recovery of uranium.

These and other objects will be apparent to those skilled in the art from the following description and accompanying drawing which is a diagrammatic sketch of a beneficiation process in accordance with the present invention.

Now it has been discovered that the asphaltite ore materials can be subjected to ore flotation operations in the absence of collectors and the gangue depressed so that a beneficiated uranium-bearing bitumen concentrate may be recovered.

The method as applied to dolomitic ore such as is found in New Mexico and Utah, for example a limestone ore impregnated with between about 1% and about 2% of bitumen, consists of crushing or grinding the ore to liberate the bitumen fraction, recovering an aqueous pulp, aerating the pulp with or without frother material present; or alternatively first aerating the pulp without frother present followed by treatment in the presence of frother material, conditioning the flotation concentrate with dispersant for nullifying the effect of contaminants on the limestone gangue, and subjecting the treated concentrate to aeration and agitation to separate limestone gangue from the final bitumen flotation concentrate. By frother material is meant a foam forming agent such as the alcohol, isobutyl carbinol or foam forming agent plus froth modifiers such as the frother pine oil plus the modifier such as fuel oil.

Run of the mine ore as received is subjected to jaw crushing, cone crushing, rod milling and sizing operations to produce a pulp having particles of a size generally smaller than about 10 mesh or about 20 mesh.

The mesh of grind for sizing may shift somewhat depending upon the mesh size for liberation of the particle mixture, but the mesh of grind will seldom be coarser than above 4 mesh or finer than about 100 mesh.

5 The pulp of, for example, —20 mesh size particles is dewatered to the proper pulp density for conditioning, if it is to be reagentized, in suitable equipment such as Dorr classifiers, cyclones, Akins classifiers, and the like. Pulp is concentrated to a solids content generally in the 10 range between about 55% and about 75% solids by weight, and preferably to between about 60% and about 70% by weight.

If the pulp is to be subjected to agitation and aeration without reagentizing, then the dilute pulp is passed to 15 flotation apparatus or concentrated pulp is diluted to a solids content of about 20% to about 40% by weight, preferably to between about 25% and about 30% by weight. Generally, it is desirable for this flotation operation that the slurry be at or near neutrality, preferably at a pH in the range between about 5 and about 9.

If a reagentized type flotation is to be effected, the frother material may be added to the dilute pulp, but preferably is added to a thick pulp. Effective frothers for this operation are hydrocarbons, such as fuel oil; alcohols, 25 such as straight chain aliphatic alcohols of between about 4 and about 8 carbon atoms, for example, isobutyl carbinol hexyl alcohol and the like; and cyclic alcohols such as the terpineols, more commonly used in an impure form known as pine oil. Such frothing materials may be used 30 individually or in mixtures, and are known in the trade by their chemical names or sold under tradenames such as American Cyanamid's "Aerofroth" mixtures, Sharples' "Pentasol 23," and the like.

Flotation of the bituminous material may be carried 35 out in suitable apparatus such as Fagergren or Denver flotation machines, or equivalent apparatus arranged so as to have one or more separation stages.

From the flotation operation wherein the slurry is agitated and aerated there is recovered a bituminous concentrate and a basically dolomite tail. The tail product usually is discarded. The concentrate from the first or rougher flotation is usually subjected to a cleaner or a second flotation operation with or without change in the reagent conditions. Concentrate from this preliminary separation 45 operation is subjected to treatment with dispersants, one of whose purposes is to clean the gangue material surfaces of contaminants so that upon subjecting the concentrate to flotation subsequently the gangue will be depressed giving a cleaner or purer concentrate product.

50 Treatment with dispersants generally consists of scrubbing the concentrate in a relatively heavy slurry form, i.e., between about 50% and about 75% solids concentration, with agents such as sodium silicate, sodium hexametaphosphate, quebracho extract, and the like, utilizing quantities of dispersants of the order of about 1 to about 20 pounds per ton of dry solids.

After agitating the concentrated slurry in a conditioning tank, the slurry is partially freed of dispersants by dewatering and washing operations. This rougher or 55 cleaner concentrate is subjected to one or more stages of recleaner operation to produce a final flotation concentrate. Feed to this recleaner operation consists generally of concentrated slurry adjusted to a solids content of the order of about 20% to about 30% solids. Tail products from the ore cleaner operation may be discarded; or if high enough in  $U_3O_8$  content the tail product may be recycled, for example, to a prior flotation stage, for example, to the rougher. The invention will be more clearly understood from the following example which is given by way of illustration and without any intention that the invention be limited thereto.

*Example I*

Uranium-bearing asphaltite limestone from New Mexico had the following analysis:

|                  | Percent by weight |
|------------------|-------------------|
| Dolomite         | 96                |
| Asphaltite       | 1.5 to 2          |
| Quartz           | 1                 |
| Mica             | 1                 |
| $U_3O_8$ content | 0.037             |

This ore was crushed, ground and size to produce a flotation feed approximately 100% of which passed through a 20 mesh standard screen. The -20 mesh material was mixed with water to produce a slurry of approximately 65% by weight solids content. The slurry was divided into four equal portions, A, B, C and D. Portion A after agitation in a conditioning tank for five minutes was diluted to a solids content of approximately 30% and introduced into a Denver subaeration flotation machine. For each 1000 parts by weight of dry solids fed to the flotation operation there was recovered 14 parts by weight of dry solids in the overflow or concentrate product. This concentrate analyzed 0.76%  $U_3O_8$ , which represents a recovery of approximately 30% of the  $U_3O_8$  present in the feed.

*Example II*

Portion B from Example I was agitated in the same conditioning tank for 5 minutes after there was added to the slurry 0.04 pound per ton of solids of pine oil. After conditioning, the conditioned concentrate was introduced into the same Denver subaeration flotation machine. For each 1000 parts by weight of dry solids feed there was recovered as a concentrate or overflow product 34 parts by weight of solids. This concentrate contains 0.67%  $U_3O_8$ , which represents a recovery of approximately 65% of the  $U_3O_8$  present in the feed.

*Example III*

Portion C from Example I was introduced into the conditioning tank and 0.07 pound per ton of dry solids of pine oil and 0.6 pound per ton of Bunker C fuel oil were added. After agitation for 5 minutes, the conditioned slurry was diluted to a solids content of approximately 30% and introduced into the same Denver subaeration flotation machine. For each 1000 parts by weight of dry solids fed to the machine there was recovered 68 parts by weight of dry solids as a concentrate. This concentrate contained 0.44%  $U_3O_8$ , which represents a recovery of approximately 86% of the  $U_3O_8$  in the feed. This concentrate was introduced into the conditioning tank of Example I and 5 pounds of sodium hexametaphosphate added per ton of dry solids. After 5 minutes' agitation in the conditioning tank the scrubbed slurry was dewatered and washed in an Akins type classifier. The washed solids were slurried with water to have a solids content of approximately 30%, and the slurry was then floated in the same Denver subaeration flotation machine. For each 1000 parts by weight of dry solids fed to the initial flotation operation there was recovered 10 parts by weight of dry solids. This final concentrate contained 2.3%  $U_3O_8$ , which represents a recovery of approximately 70% of the  $U_3O_8$  in the original feed. By drying and igniting this flotation concentrate in a muffle furnace a product assaying approximately 22%  $U_3O_8$  was produced.

Having thus described the invention what I claim is:

1. A method for the beneficiation of uranium-bearing asphaltite ore which comprises comminuting the ore to liberation of the bituminous constituents, converting the liberated ore to an aqueous pulp and agitating and aerating the pulp in the absence of a collector to effect flotation of a bituminous concentrate, scrubbing the concentrate in slurry form with dispersants for bituminous material, washing the scrubbed slurry free of contaminants and

dispersants and aerating and agitating the scrubbed concentrate in the absence of a collector to effect flotation and to recover a second bituminous concentrate containing the uranium constituents.

- 5 2. A method for the beneficiation of uranium-bearing asphaltite ore which comprises comminuting the ore to liberation of the bituminous constituents, converting the liberated ore to an aqueous pulp, conditioning the aqueous pulp in the absence of a collector with frother material, 10 agitating and aerating the pulp to effect flotation of a bituminous concentrate, scrubbing the concentrate in slurry form with dispersants for bituminous material, washing the scrubbed slurry free of contaminants and dispersants and aerating and agitating the scrubbed concentrate in the absence of a collector to effect flotation and to recover a second bituminous concentrate containing the uranium constituents.
- 15 3. A method for the beneficiation of uranium-bearing asphaltite ore which comprises comminuting the ore to liberation of the bituminous constituents, converting the liberated ore to an aqueous pulp and agitating and aerating the pulp in the absence of a collector at a pH in the range between about 5 and about 9 to effect flotation of a bituminous concentrate, scrubbing the concentrate in 20 slurry form with dispersants for bituminous material, washing the scrubbed slurry free of contaminants and dispersants and aerating and agitating the scrubbed concentrate in the absence of a collector to effect flotation and to recover a second bituminous concentrate containing the uranium constituents.
- 25 30 4. A method for the beneficiation of uranium-bearing asphaltite impregnated limestone which comprises comminuting the ore to liberation of the bituminous constituents, converting the liberated ore to an aqueous pulp, conditioning the aqueous pulp with frother material, agitating and aerating the pulp in the absence of a collector to effect flotation of a bituminous concentrate, scrubbing the concentrate in slurry form with dispersants for bituminous material, washing the scrubbed slurry free of contaminants and dispersants and aerating and agitating the scrubbed concentrate in the absence of a collector to effect flotation and to recover a second bituminous concentrate containing the uranium constituents.
- 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960

of pine oil per ton of dry solids, agitating and aerating the pulp in the absence of a collector to effect flotation of a bituminous concentrate, scrubbing the concentrate in slurry form with between about 5 pounds and about 10 pounds of sodium hexametaphosphate per ton of dry solids, washing the scrubbed slurry free of contaminants and sodium hexametaphosphate and aerating and agitating the scrubbed concentrate in the absence of a collector to effect flotation and to recover a second bituminous concentrate.

8. A method for the beneficiation of uranium-bearing asphaltite impregnated limestone which comprises comminuting the ore to a size such that the largest particles fall in the range between about 10 mesh and about 20 mesh, converting the comminuted ore to an aqueous pulp, conditioning the aqueous pulp with about 0.07 pound of pine oil per ton of dry solids and about 0.6 pound of Bunker C fuel oil per ton of dry solids, agitating and aerating the pulp in the absence of a collector to effect flotation of a bituminous concentrate, scrubbing the concentrate in slurry form with between about 5 pounds and about 10 pounds of sodium hexametaphosphate per ton of dry solids, washing the scrubbed slurry free of contaminants and sodium hexametaphosphate and aerating and agitating the scrubbed concentrate in the absence of a collector to effect flotation and to recover a second bituminous concentrate.

9. A method for the beneficiation of uranium-bearing asphaltite impregnated limestone which comprises comminuting the ore to a size such that the largest particles fall in the range between about 10 mesh and about 20 mesh, converting the comminuted ore to an aqueous

pulp, conditioning the aqueous pulp with about 0.07 pound per ton of pine oil and about 0.6 pound per ton of Bunker C fuel oil, agitating and aerating the pulp in the absence of a collector to effect flotation of a bituminous concentrate, scrubbing the concentrate in slurry form with between about 5 pounds and about 10 pounds of sodium hexametaphosphate per ton of dry solids, washing the scrubbed slurry free of contaminants and sodium hexametaphosphate, aerating and agitating the scrubbed concentrate in the absence of a collector to effect flotation and to recover a second bituminous concentrate, and igniting the bituminous second concentrate to produce a further beneficiated concentrate.

15

References Cited in the file of this patent

UNITED STATES PATENTS

|           |            |                |
|-----------|------------|----------------|
| 1,454,838 | Borcherdt  | May 8, 1923    |
| 2,130,144 | McClave    | Sept. 13, 1938 |
| 2,161,010 | Breerwood  | June 6, 1939   |
| 2,363,315 | Grothe     | Nov. 21, 1944  |
| 2,389,727 | Herkenhoff | Nov. 27, 1945  |
| 2,469,422 | Weinig     | May 10, 1949   |
| 2,507,012 | Heilmann   | May 9, 1950    |
| 2,594,929 | Howell     | Apr. 29, 1952  |

OTHER REFERENCES

Denver Equipment Company Handbook, 1954, Denver  
30 Equipment Company, pages 582-609.  
Taggart: Handbook of Mineral Dressing, 1945, pages  
12-35.

UNITED STATES PATENT OFFICE  
CERTIFICATE OF CORRECTION

Patent No. 2,973,864

March 7, 1961

Phillip E. McGarry

It is hereby certified that error appears in the above numbered patent requiring correction and that the said Letters Patent should read as corrected below.

Column 1, line 20, for "imprognated" read -- impregnated  
--; column 4, line 9, strike out "in the absence of a collector"  
and insert the same after "pulp" in line 10, same column;  
line 64, strike out "and sodium".

Signed and sealed this 19th day of September 1961.

(SEAL)

Attest:

ERNEST W. SWIDER

Attesting Officer

DAVID L. LADD

Commissioner of Patents

USCOMM-DC